

March 10, 1942.

J. C. VIGNOS

2,276,074

METHOD OF MAKING FERRO-ALLOYS

Filed Jan. 23, 1941



INVENTOR.

James C. Vignos  
BY Brown, Crittell & Ellicott  
His ATTORNEYS.

## UNITED STATES PATENT OFFICE

2,276,074

## METHOD OF MAKING FERRO-ALLOYS

James C. Vignos, Canton, Ohio, assignor to Ohio  
Ferro-Alloys Corporation, Philo, Ohio, a cor-  
poration of Ohio

Application January 23, 1941, Serial No. 375,593

14 Claims. (Cl. 75—56)

This invention relates to methods of making silicon-containing ferro-alloys of carbide-forming metals such, for example, as chromium and manganese, and particularly to those for use in producing low carbon ferrous base alloys of such metals, especially stainless irons and steels.

The word "ferro-alloys" is used by metallurgists to designate alloys of iron with such large contents of one or more alloying elements, other than carbon, that they are used for introducing those elements in the production of alloy irons and steels. This term and the alloys comprehended by it are well understood in the art.

The invention is desirably applicable to the production of ferro-alloys of low carbon content, and may therefore be described with particular reference thereto. For the production of certain ferrous base alloys the carbon content of the ferro-alloys used is highly important. For instance, it is well recognized that in the production of various ferrous base alloys containing chromium, and particularly in the production of stainless irons and steels, it is essential that the ferro-chrome used be of extremely low carbon content. Such ferro-alloys may therefore be referred to herein as exemplifying, but not limiting, the ferro-alloys of the carbide-forming elements with which the invention is concerned.

In the production of stainless irons and steels, for example, the common practice is to react a ferro-alloy of silicon and chromium, i. e., ferro-chrome-silicon, with chrome ore to produce the desired final alloy. The carbon content of the final alloy is definitely a function of that of the ferro-alloy used, and where the carbon of the product is important there are used ferro-alloys of exceedingly low carbon content. For example, U. S. Patent No. 1,925,886, issued on an application filed by me, refers to the use of a ferrochrome-silicon alloy containing 46 per cent of chromium, 35.64 per cent of silicon, and but 0.32 per cent of carbon. Generally speaking, the patents in this field refer to the use of ferro-chrome-silicon alloys of much lower carbon content. Thus, U. S. Patent No. 2,176,686 to M. J. Udy gives an example of the use of such an alloy containing 25.2 per cent of chromium, 40 per cent of silicon, and only 0.05 per cent of carbon, while that patentee in his companion Patent No. 2,176,687 discloses the use of a similar alloy containing 50 per cent of silicon, 23.4 per cent of chromium, and 0.04 per cent of carbon.

Because no other practical way of making such ferro-alloys with such low content of carbon has been known, most of the ferrochrome-silicon alloys used for these purposes have been produced by direct reduction of ore. In the case of ferro-chrome this is done by reducing a charge of quartz and chrome ore with carbon, for example

as disclosed in Patent No. 891,898 to F. M. Becket.

The belief in the art has been that the carbon content of all ferrochrome-silicon alloys is a function of the silicon content, the carbon being lowered, at least up to a certain point, as the silicon content is increased. This relationship is described in U. S. Patent No. 1,567,898 to F. M. Becket, and the accompanying drawing 10 is a reproduction of the graph given in that patent as representing the carbon-silicon relationship. As appears therefrom, and as described in the specification of the patent, in ferrochrome-silicon alloys the carbon content of the alloy decreases rapidly as the silicon content increases from about 17 to about 40 per cent, while further increase in the silicon content up to about 67 per cent results in little or no further decrease in the carbon content. According to the patent 15 it is preferred to use between 40 and 50 per cent of silicon, corresponding to a carbon range of approximately 0.1 to 0.04 per cent. Included in this drawing are a number of points representing the silicon and carbon contents of low carbon ferrochrome-silicon and ferromanganese-silicon alloys in accordance with the present invention.

The prior direct reduction processes require 20 careful control at electric furnace temperatures, which makes operation difficult, and the economics of the process causes the cost of the products to be considerably out of line in comparison with ferro-alloys of higher carbon content. This results, at least in part, in the high cost of stainless irons and steels.

Other ferro-alloys of carbide-forming elements 25 appear to respond to the same general relationship just described. For instance, the commercial grades of ferromanganese-silicon alloys show the same general effect of silicon on the carbon content, as appears from the four following commercial grades:

| Manganese | Silicon | Carbon  |
|-----------|---------|---------|
| Percent   | Percent | Percent |
| 65-70     | 20-25   | 1 1.0   |
| 65-70     | 16-20   | 2.0     |
| 65-70     | 14-18   | 2.5     |
| 65-70     | 12-14   | 2 3.0   |

50 1 Maximum.

2 Approximate.

A major object of the present invention is to 55 provide ferro-alloys of silicon and carbide-forming elements which are of lower carbon content for any given silicon content than similar alloys produced by direct reduction methods, and to do so easily and at lower cost than heretofore.

A further object is to easily, cheaply and simply convert high carbon grades of ferro-alloys of carbide-forming elements, especially chromium

and manganese, into lower carbon ferro-alloys containing silicon for use as intermediate materials in producing alloy irons and steels.

Yet another object is to provide a method of producing low carbon ferro-alloys of silicon and carbide-forming elements, particularly ferro-chrome-silicon and ferromanganese-silicon alloys, which proceeds from ordinary, cheap, high carbon ferro-alloys, which is easily practiced and whose products are less expensive than the same grades of the same ferro-alloys now available on the market, and which produces ferro-alloys that are both of sufficiently low carbon content for producing low carbon ferrous base alloys and also of lower silicon content than has heretofore been produced with such carbon contents.

Still another object is to provide low carbon ferro-alloys of the type referred to in which the carbon content is below that of alloys of the same silicon content produced by direct ore reduction, which are cheap, easily produced, and satisfactory for all purposes for which similar alloys produced by direct ore reduction are used.

These and other objects of my invention are attained in the manner now to be described.

The invention is predicated upon my discovery that, contrary to the belief expressed above, the carbon content of ferrochrome-silicon and similar ferro-alloys containing silicon is not directly or strictly dependent upon the silicon content, and that in simple and easy fashion these alloys may be made with carbon contents below those to be expected for a given silicon content based upon the relationship previously accepted in the art and expressed in U. S. Patent No. 1,567,898. In accordance with the present invention this is accomplished by reacting a high carbon grade of the desired ferro-alloy, ferrosilicon, and an oxidizing agent. In the practice of the invention the oxidizing agent serves primarily to oxidize the carbon and so lower its content to a point appreciably below that which would be expected for the silicon content of the product. The action of the oxidant is exothermic so that large amounts of heat are liberated, which desirably contributes to the economics of the process. In this manner there is produced a ferrosilicon alloy of the carbide-forming element present in the high carbon ferro-alloy which is of the low carbon content necessary for the production of such low carbon alloys as stainless irons and steels, and which may either contain less silicon than has been present in ferro-alloys of the same carbon grades, or less carbon for a given silicon content.

The invention may be practiced in various ways but to effect reaction between the carbon oxidizing agent and the carbon it is necessary that at least the ferro-alloy or the ferrosilicon be molten. By way of example and not of limitation, the high carbon ferro-alloy, such as high carbon ferrochromium produced by direct ore reduction, may be mixed with the oxidizing agent and the mixture added to molten ferrosilicon. Alternatively, the ferrosilicon and the oxidizing agent may be mixed and added to molten high carbon ferrochrome or other ferro-alloy of a carbide-forming element. Yet another possible procedure is to mix molten ferrosilicon and molten high carbon ferro-alloy in the presence of the oxidizing agent, or to add the oxidizing agent to a pre-formed mixture of the two. The high carbon ferro-alloy and the ferrosilicon produce the desired ferro-alloy-silicon.

Various oxidizing agents capable of oxidizing

carbon at a temperature at which one of the reactants is molten may be used such, for example, as nitrates, chlorates, perborates, persulfates, permanganates, and the like, especially those of the alkali metals, preference being given, of course, to the sodium salts because they are more commonly available and usually cheaper than the other alkali metal salts.

Proportions of the three reactants applicable to all starting materials and products can not be given, of course, because these will depend upon the particular content of carbide-forming alloying element and silicon desired in the product and this will in turn depend upon the concentrations of alloying element in the high carbon ferrochrome or other ferro-alloy and of silicon in the ferrosilicon used. Likewise, the amount of oxidizing agent used will depend upon the particular agent used, the content of carbon in the ferro-alloy, and the carbon content desired in the product. However, it may be stated that, generally speaking, the two ferro-alloys are mixed in proportions such as to give the desired content of silicon and alloying element in the product, and the oxidizing agent is used in an amount such as to effect the desired reduction in carbon content. Also, as further guides to the practice of the invention, it may be said that with ordinary high carbon ferro-alloys, such as those produced by direct ore reduction, it is advantageous to use ferro-silicon containing at least about 40 per cent of silicon. These two alloys should be proportioned so that the ferro-alloy-silicon product contains the desired amount of alloying element, in any event in excess of 5 per cent thereof, together with at least about 10 per cent of silicon. Desirably, the silicon will not exceed about 40 per cent in the finished ferro-alloy. The high carbon ferro-alloys used may be those produced by direct ore reduction because they may be made cheaply and easily. Such ferro-alloys may, of course, contain silicon due to the use of ores containing it, or to addition of silica to the furnace burden, which is desirable both because the presence of silicon lowers the melting point of the ferro-alloy, and also because the silicon-containing ferro-alloys crush more easily.

For low carbon products the oxidant should be used in an amount such that the final alloy contains not over about 0.15 per cent of carbon, although much lower contents may be produced, as will appear hereinafter.

The practicability of the invention in producing low carbon ferro-alloy-silicon alloys, particularly those of substantially lower silicon content for a given carbon content than have been available heretofore, has been demonstrated by the extensive production of such alloys on a tonnage, or commercial basis. Examples from actual practice of ferrochrome-silicon alloys appear in the following table:

| Alloy No. | Carbon  | Silicon | Chrome  |
|-----------|---------|---------|---------|
|           | Percent | Percent | Percent |
| 1.        | 0.04    | 39.58   | 34.78   |
| 2.        | 0.07    | 35.88   | 16.15   |
| 3.        | 0.06    | 37.54   | 17.90   |
| 4.        | 0.12    | 33.14   | 20.60   |
| 5.        | 0.04    | 36.43   | 17.93   |
| 6.        | 0.02    | 36.55   | 16.23   |
| 7.        | 0.05    | 31.40   | 22.75   |
| 8.        | 0.01    | 38.36   | 17.33   |
| 9.        | 0.14    | 30.11   | 26.65   |
| 10.       | 0.06    | 31.40   | 23.50   |
| 11.       | 0.11    | 27.10   | 29.10   |
| 12.       | 0.07    | 34.93   | 18.90   |

Alloy No. 1 was produced by mixing ferro-chrome containing 5.25 per cent of carbon and 69 per cent of chromium with 10 per cent by weight of sodium nitrate and adding it to molten 78 per cent ferrosilicon. According to the carbon-silicon relationship described in Patent No. 1,567,898 and shown in the accompanying drawing the resultant alloy should have contained approximately 0.125 per cent of carbon, whereas the actual content was 0.04 per cent, which illustrates clearly the profound effect of the oxidizing agent when used in accordance with this invention.

Alloy No. 2 was made by adding high carbon ferrochromium and sodium nitrate to molten 50 per cent ferrosilicon. According to the graph of Patent No. 1,567,898 this alloy should have contained about 0.2 per cent of carbon. The other alloys were made in similar fashion, and it will be observed in each instance that the carbon content is below that which would have been expected.

Examples of ferromanganese-silicon alloys produced in accordance with the invention are shown in the following table:

| Alloy No. | Carbon  | Silicon | Manganese |
|-----------|---------|---------|-----------|
|           | Percent | Percent | Percent   |
| 13.....   | 0.02    | 30.00   | 25.10     |
| 14.....   | 0.02    | 33.15   | 27.51     |
| 15.....   | 0.03    | 27.74   | 26.33     |

These were made by adding mixtures of high carbon ferromanganese and oxidizing agent, such as sodium nitrate, to molten ferrosilicon.

The carbon and silicon contents of alloys Nos. 1 to 15 are represented by x's in the accompanying drawing. It will be observed that in all of these alloys produced in accordance with the invention the carbon content for any given silicon content is below that which would be expected according to existing belief in the art or produced by the direct reduction methods used heretofore.

These alloys may be used for the purposes and in the same manner as other ferro-alloys. Moreover, the difference in carbon content is so marked in every case that when the alloys provided by the invention are reacted with a metallic oxide, ore, or partially reduced ore, with or without an oxidizing agent, the resulting ferrous base alloy, such as stainless iron or steel, is of much lower carbon content than could be produced heretofore from the available ferro-alloys containing the normal carbon content for a given silicon content. The term "partially reduced ore" as used herein has reference to ore which has been subjected to reduction, by means of carbon or a reducing gas, to convert at least a portion, for instance more than 2 per cent, of the metallic oxide to the metallic state.

The invention has been described with particular reference to the production of ferro-alloy-silicons of very low carbon content. However, from what has been said it will be understood that the gist of the invention resides in providing such alloys in which the carbon content for a given silicon content is less than that obtainable by direct reduction of ore and below that which would be expected according to prior art beliefs. Hence the carbon content, within the limitation just stated may be such as it requisite to the use to which the product is to be put, i. e., it may be exceedingly low or rela-

tively high but in all cases it lies below the graph shown in the accompanying drawing. For instance, to make a ferrochrome-silicon for use in making stainless ferrous base alloys there may be used a ferrochrome produced by direct reduction of ore to contain about 20 per cent of silicon. According to the graph this will contain 2.5 per cent of carbon. This is then reacted with ferrosilicon and oxidant to produce a ferro-chrome-silicon with 40 to 50 per cent of silicon and 0.01 to 0.02 per cent of carbon. In like fashion there may be made products containing less than 0.1 per cent of carbon at 40 per cent of silicon, less than 0.25 per cent of carbon at 35 per cent of silicon, not over about 0.5 per cent of carbon at 30 per cent of silicon, not over 1.25 per cent of carbon at 25 per cent of silicon, etc., the carbon content in any given case lying below the curve shown in the drawing.

According to the provisions of the patent statutes, I have explained the principle and method of practicing my invention and have described what I now consider to represent its best embodiments. However, I desire to have it understood that, within the scope of the appended claims, the invention may be practiced otherwise than as specifically described.

I claim:

1. That method of producing a low carbon ferro-alloy of silicon and a carbide-forming metal from a higher carbon ferro-alloy of said metal produced by direct reduction, ferrosilicon, and an oxidizing agent as reactants which comprises providing at least one of said ferro-alloys in molten condition and mixing therewith the other said reactants and by the reaction producing a ferro-alloy of substantially decreased carbon content.

2. That method of producing a low carbon ferro-alloy of silicon and a carbide-forming metal from a higher carbon ferro-alloy of said metal produced by direct reduction, ferrosilicon, and an alkali metal nitrate as reactants which comprises providing at least one of said ferro-alloys in molten condition and mixing therewith the other said reactants and by the reaction producing a ferro-alloy of substantially decreased carbon content.

3. A method of producing a low carbon ferro-alloy of silicon and a carbide-forming metal according to claim 1 in which said ferrosilicon contains more than about 40 per cent of silicon, and said oxidant is sodium nitrate.

4. A method according to claim 1 in which said carbide-forming metal is of the group consisting of chromium and manganese and said ferrosilicon contains more than about 40 per cent of silicon.

5. That method of producing a low carbon ferro-alloy of silicon and a carbide-forming metal from a higher carbon ferro-alloy of said metal produced by direct reduction, ferrosilicon containing at least about 40 per cent of silicon, and an oxidizing agent as reactants which comprises providing at least one of said ferro-alloys in molten condition and mixing therewith the other said reactants and thereby producing said low carbon ferro-alloy, the amount of said agent being such that the ferro-alloy product contains carbon in an amount less for a given silicon content than is producible in the same alloy made by direct reduction.

6. That method of producing a low carbon ferro-alloy according to claim 5, said carbide-forming metal being of the group consisting of

chromium and manganese, said ferrosilicon containing at least about 40 per cent of silicon, and said oxidizing agent being an alkali metal nitrate and being used in an amount such that the ferro-alloy product contains not over about 0.25 per cent of carbon.

7. That method of producing a low carbon ferro-alloy of silicon and a carbide-forming metal from a higher carbon ferro-alloy of said metal produced by direct reduction, from ferrosilicon and an oxidizing agent as reactants which comprises providing at least one of said ferro-alloys in the molten state and then adding the other said reactants and thereby by reaction producing said low carbon ferro-alloy, said materials being so proportioned that the ferro-alloy product contains more than about 5 per cent of said carbide-forming metal, at least about 10 per cent of silicon, the remainder being chiefly iron, and carbon in an amount which for the silicon present is less than contained in the same alloy produced by direct reduction.

8. That method of producing a low carbon ferrochrome-silicon from high carbon ferrochrome produced by direct reduction, ferrosilicon, and a carbon oxidant as reactants which comprises providing at least one of said ferro-

alloys in molten condition and mixing therewith the other said reactants and by reaction producing low carbon ferrochrome silicon alloy.

9. That method of producing a low carbon ferromanganese-silicon from high carbon ferromanganese produced by direct reduction, ferrosilicon, and an oxidizing agent as reactants which comprises providing at least one of said ferro-alloys in molten condition and mixing the other reactants therewith and by reaction thereof producing said low carbon ferro-alloy.

10. A method according to claim 2, said ferrosilicon containing at least about 40 per cent of silicon.

11. A method according to claim 2, said nitrate being sodium nitrate.

12. A method according to claim 7, said agent being an alkali metal nitrate.

13. A method according to claim 7, said ferrosilicon containing at least about 40 per cent of silicon.

14. A method according to claim 7, said ferrosilicon containing at least about 40 per cent of silicon, said ferro-alloy being selected from the group consisting of ferrochrome and ferromanganese, and said agent being sodium nitrate.

JAMES C. VIGNOS.